# EUROPEAN PATENT SPECIFICATION

(11) **EP 0 349 331 B1**
(45) Date of publication and mention of the grant of the patent: **22.03.1995**
(21) Application number: 89306645.6
(22) Date of filing: 30.06.1989
(51) Int. Cl.: G03C 7/305, G03C 7/34

(54) **Color photographic material**
Farbphotographisches Material
Materiau photographique couleur

(30) Priority: 30.06.1988 US 213415
(43) Date of publication of application: 03.01.1990
(73) Proprietor: EASTMAN KODAK COMPANY (a New Jersey corporation), Rochester, New York 14650 (US)
(72) Inventor: Szajewski, Richard Peter c/o EASTMAN KODAK CO., Rochester New York 14650 (US); Taber, Terry Ray c/o EASTMAN KODAK CO., Rochester New York 14650 (US)
(74) Representative: Baron, Paul Alexander Clifford

(56) References cited:
- EP-A- 0 271 324
- GB-A- 2 072 363

## Description

This invention relates to color photographic elements. In a particular aspect, it relates to color photographic elements with a particular combination of development inhibitor releasing compound and cyan dye-forming coupler.

Photographic couplers which release a development inhibitor in a controlled manner are described in U.S. Patents 4,248,962 and 4,409,323, inter alia. These couplers comprise a coupler moiety which has a timing group joined in its coupling position. A development inhibitor is attached to the timing group and is released from it after the bond between the timing group and the coupler is cleaved as a result of reaction between the coupler and oxidized color developing agent. Mechanisms by which such release of the development inhibitor from the timing group can occur include an intermolecular nucleophilic displacement reaction, an electron transfer reaction, and a hydrolysis reaction. Development inhibitors also can be released, as a function of development, from timing groups which are released from compounds which are not couplers such as the hydrazides of U.S. Patent 4,684,604 and the hydroquinones of European Patent Application 0,167,168.

One of the advantageous effects obtained as a result of release of a development inhibitor, either directly from a coupler or other carrier moiety, or through a timing group as described above, is an improvement in sharpness of the resulting photographic image.

Also known are cyan dye-forming image couplers that contain a ureido group in the 2-position.

Lau, U.S. Patent 4,333,999 issued June 8, 1982, describes cyan dye-forming couplers containing p-cyanophenylureido substituents in the 2-position of the coupler. These couplers are described as yielding dyes having desirable hues and good stability properties.

U.S. Patent 4,775,616 issued October 4, 1988, describes couplers which improve upon those described in the ′999 patent by modifying the 5-position substituent. The ′999 and ′616 patents suggest the use of the cyan couplers therein described in combination with DIR couplers, but do not specifically suggest that they be used with couplers of the type described in the ′962 or ′323 patents.

U.S. Patents 4,434,225 and 4,609,619 describe phenolic cyan dye-forming couplers containing a ureido group in the 2-position. Use of one of these couplers with a DIR coupler is mentioned in these patents. However, they do not describe any particular combination of phenolic coupler and DIR coupler nor the particular advantage deriving from the selection of the present invention.

It would be desirable to provide color photographic materials which have improved sharpness.

We have found that unexpected improvements in sharpness can be obtained with a photographic element comprising a support bearing a silver halide emulsion layer having associated therewith a DIR compound having the structure I:
wherein:
CAR is a carrier moiety,
TIME is a timing group and
INH is a development inhibitor moiety; together with a cyan dye-forming coupler having the structure II:
wherein:
m is 0 or 1;
n is 0, 1 or 2;
Y is halogen, or sulfonyl;
Q is -O- or -NH-;
R¹ is an unsubstituted or a substituted, straight or branched chain alkyl group having from 1 to 20 carbon atoms, an unsubstituted or a substituted cycloalkyl group having from 3 to 8 carbon atoms in the ring, an alkylcarbonyl or an alkoxycarbonyl group having from 1 to 20 carbon atoms in the alkyl or the alkoxy moiety;
R² is as defined for R¹ or is hydrogen;
R³ is an unsubstituted or a substituted alkyl group having from 1 to 24 carbon atoms, an unsubstituted or a substituted cycloalkyl group having from 3 to 8 carbon atoms in the ring, an unsubstituted or a substituted aryl group having from 6 to 24 carbon atoms, or an unsubstituted or a substituted heterocyclic group having from 3 to 8 atoms in the heterocyclic ring, wherein the hetero ring atoms can be nitrogen, oxygen, or sulfur;
when R³ is a primary alkyl group, R¹ contains at least 2 carbon atoms;
Z is hydrogen or a coupling-off group; and
the -CN substituent on the phenyl ureido group is para or meta to the ureido group.

When the R¹ and R² groups are substituted, such substituents include hydroxy, halogen, or alkoxy having from 1 to 8 carbon atoms.

When the R³ group is substituted, such substituents include alkyl, aryl, alkoxy, aryloxy, alkylthio, arylthio, hydroxy, halogen, alkoxycarbonyl, aryloxycarbonyl, carboxy, acyl, acyloxy, carbonamido, carbamoyl, alkylsulfonyl, arylsulfonyl, sulfonamido and sulfamoyl groups wherein the alkyl and aryl substituents, and the alkyl and aryl moieties of the alkoxy, aryloxy, alkylthio, arylthio, alkoxycarbonyl, arylcarbonyl, acyl, acyloxy, carbonamido, carbamoyl, alkylsulfonyl, arylsulfonyl, sulfonamido and sulfamoyl substituents can contain, respectively, from 1 to 10 carbon atoms and from 6 to 30 carbon atoms and can be further substituted with such substituents.

Coupling off groups defined by Z are well known to those skilled in the art.

Representative classes of coupling-off groups include alkoxy, aryloxy, heteroyloxy, sulfonyloxy, acyloxy, acyl, heterocyclyl, sulfonamido, phosphonyloxy and arylazo. These coupling-off groups are described in the art, for example, in U.S. Patent Nos. 2,455,169; 3,227,551; 3,432,521; 3,476,563; 3,617,291; 3,880,661; 4,052,212 and 4,134,766; and in U.K. Patents and published application Nos. 1,466,728; 1,531,927; 1,533,039; 2,006,755A and 2,017,704A.

Examples of suitable coupling-off groups which can be represented by Z are:
-OCH₃, -OC₆H₅, -OCH₂CONHCH₂CH₂OH, -OCH₂CONHCH₂CH₂OCH₃, -OCH₂CONHCH₂CH₂OCOCH₃,
-OCH₂CH₂NHSO₂CH₃,
and
Especially preferred Z groups are hydrogen and
where R⁴ is an alkyl or an alkoxy group having from 1 to 10 carbon atoms.

While improvements in sharpness are obtained when couplers of Structure II, above, are used in combination with DIR compounds of Structure I above, especially advantageous effects are obtained with the following preferred couplers of Structure II.

In a preferred embodiment the cyano group is in the para position with respect to the ureido group and n is 0.

In a particular preferred embodiment, n is 0, the cyano group is para to the ureido group, R¹ is alkyl of 1 to 20 carbon atoms and R² is hydrogen or alkyl of 1 to 4 carbon atoms.

In an especially preferred embodiment, n is 0, the cyano group is para to the ureido group, R¹ is alkyl of 1 to 14 carbon atoms, R² is hydrogen and R³ is alkyl of 2 to 24 carbon atoms.

The DIR compounds which satisfy Structure I are known in the art and are described in such patents as U.S. Patent 4,248,962; 4,409,323; 4,684,604; 4,737,451; U.K. Patent Application 2,099,167; and EP Published Applications 167,168 and 255,085, as well as in U.S. Patents 4,546,073; 4,564,587; 4,618,571; 4,698,297; and OLS 3,307,506. Other useful DIR compounds are described in DeSelms and Kapecki U.S. Patent 4,782,012, issued November 1, 1988; Szajewski, Poslusny and Slusarek U.S. Patent Application Serial No. 209,741, filed June 21, 1988; and Begley, Carmody and Buchanan U.S. Patent Applications 213,416 and 214,090, both filed June 30, 1988.

The carrier moiety, represented by CAR, can be any moiety which, as a result of reaction with oxidized color developing agent, will release the timing group. Preferably the carrier is a coupler, but it can be another group, such a hydrazide, a hydrazine or a hydroquinone. Coupler moieties can form a colored or colorless, diffusible or nondiffusible, reaction product with oxidized color developing agent. Preferred are cyan dye-forming coupler moieties.

When the carrier is a coupler moiety, the DIR compounds are DIR couplers represented by the structure
where COUP is a coupler moiety. The preferred - INH group is a mercaptotetrazole or benzotriazole inhibitor.

Preferably the DIR compound is a cyan dye-forming DIR coupler and is contained in a red-sensitive silver halide emulsion layer together with the cyan dye-forming image coupler
or the DIR compound is a yellow dye-forming DIR coupler and is contained in a red-sensitive silver halide emulsion layer together with the cyan dye-forming image coupler.
Particularly preferred are couplers where COUP is a naphtholic cyan dye-forming coupler moiety represented by the following generalized structure:
where:
the unsatisfied bond represents the point of attachment of the timing group, and
BALL is a ballast group such as aryl and alkyl, especially alkoxyaryl and aryloxyalkyl.

Also useful are compounds where COUP is a yellow dye forming coupler moiety having one of the structures
or
where
the unsatisfied bond is the point of attachment to the timing group,
BALL is a ballast group such as alkoxycarbonyl, alkoxy, alkylsulfonamido and alkylsulfamyl,
X is as defined below, and
Y is alkyl such as methyl and t-butyl, and aryl such as phenyl and alkoxy phenyl.

Preferred timing groups, represented by TIME, for use in these couplers are described in the aforementioned ′962 and ′323 patents and European Patent Application 0255085.

Particularly preferred are those timing groups which have the structures:
and
where:
p is 1 to 4;
q is 0 or 1;
A is -O- or
R⁵ is hydrogen, alkyl of 1-20 carbon atoms or aryl of 6 to 20 carbon atoms; and
X is hydrogen and one or more substituents independently selected from hydroxy, cyano, fluoro, chloro, bromo, iodo, nitro, alkyl, alkoxy, aryl, aryloxy, alkoxycarbonyl, aryloxycarbonyl, carbonamido, and sulfonamido X is preferably hydrogen, cyano, nitro or sulfonamido.

The development inhibitor which is eventually released from the DIR coupler can be any of the development inhibitors known in the art, such as mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzotriazoles, and benzodiazoles. Preferred are mercaptotetrazole inhibitors, benzotriazole inhibitors, and oxadiazole inhibitors. Particularly preferred are those inhibitors which are substituted with groups that cause them to be deactivated when they diffuse into processing solution. Such inhibitors are described in U.S. Patent 4,477,563, U.K. Patent Application 2,099,167 and U.S. Patent 4,782,012 issued November 1, 1988. Other useful inhibitors are described in Japanese Published Patent Applications 60-233650, 60-225156, 60-182438 and European Published Patent Applications 0167168, 0101621, 0192199, 0157146.

Examples of preferred couplers which satisfy structures I and II, respectively, are shown in Tables I and II below:

The compounds and couplers used in this invention are, in general, known compounds and can be prepared by techniques known in the art. Compounds, described in the copending applications referred to above on page 6 are novel and can be prepared by the procedures described in those applications.

The coupler combinations used in the elements of this invention can be incorporated in silver halide emulsions and the emulsions can be coated on a support to form a photographic element. Alternatively, one or both of the couplers can be incorporated in photographic elements adjacent the silver halide emulsion where, during development, the coupler will be in reactive association with development products such as oxidized color developing agent.

The photographic elements can be either single color or multicolor elements. In a multicolor element, the cyan dye-forming coupler is usually associated with a red-sensitive emulsion, although it could be associated with an unsensitized emulsion or an emulsion sensitized to a different region of the spectrum. Multicolor elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art.

A typical multicolor photographic element comprises a support bearing a cyan dye image-forming unit comprising at least one red-sensitive silver halide emulsion layer having associated therewith at least one cyan dye-forming coupler, a magenta image forming unit comprising at least one green-sensitive silver halide emulsion layer having associated therewith at least one magenta dye-forming coupler and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like.

In the following discussion of suitable materials for use in the elements of this invention, reference will be made to Research Disclosure, December 1978, Item 17643, published by Kenneth Mason Publications, Ltd., The Old Harbourmaster's, 8 North Street, Emsworth, Hampshire PO10 7DD, ENGLAND. This publication will be identified hereafter by the term "Research Disclosure."

The silver halide emulsions employed in the elements of this invention can be comprised of silver bromide, silver chloride, silver iodide, silver chlorobromide, silver chloroiodide, silver bromoiodide, silver chlorobromoiodide or mixtures thereof. The emulsions can include silver halide grains of any conventional shape or size. Specifically, the emulsions can include coarse, medium or fine silver halide grains. High aspect ratio tabular grain emulsions are specifically contemplated, such as those disclosed by Wilgus et al U.S. Patent 4,434,226, Daubendiek et al U.S. Patent 4,414,310, Wey U.S. Patent 4,399,215, Solberg et al U.S. Patent 4,433,048, Mignot U.S. Patent 4,386,156, Evans et al U.S. Patent 4,504,570, Maskasky U.S. Patent 4,400,463, Wey et al U.S. Patent 4,414,306, Maskasky U.S. Patents 4,435,501 and 4,643,966 and Daubendiek et al U.S. Patents 4,672,027 and 4,693,964. Also specifically contemplated are those silver bromoiodide grains with a higher molar proportion of iodide in the core of the grain than in the periphery of the grain, such as those described in GB 1,027,146; JA 54/48,521; US 4,379,837; US 4,444,877; US 4,665,012; US 4,686,178; US 4,565,778; US 4,728,602; US 4,668,614; US 4,636,461; EP 264,954. The silver halide emulsions can be either monodisperse or polydisperse as precipitated. The grain size distribution of the emulsions can be controlled by silver halide grain separation techniques or by blending silver halide emulsions of differing grain sizes.

Sensitizing compounds, such as compounds of copper, thallium, lead, bismuth, cadmium and Group VIII noble metals, can be present during precipitation of the silver halide emulsion.

The emulsions can be surface-sensitive emulsions, i.e., emulsions that form latent images primarily on the surfaces of the silver halide grains, or internal latent image-forming emulsions, i.e., emulsions that form latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent.

The silver halide emulsions can be surface sensitized. Noble metal (e.g., gold), middle chalcogen (e.g., sulfur, selenium, or tellurium), and reduction sensitizers, employed individually or in combination, are specifically contemplated. Typical chemical sensitizers are listed in Research Disclosure, Item 17643, cited above, Section III.

The silver halide emulsions can be spectrally sensitized with dyes from a variety of classes, including the polymethine dye class, which includes the cyanines, merocyanines, complex cyanines and merocyanines (i.e., tri-, tetra-, and poly-nuclear cyanines and merocyanines), oxonols, hemioxonols, styryls, merostyryls, and streptocyanines. Illustrative spectral sensitizing dyes are disclosed in Research Disclosure, Item 17643, cited above, Section IV.

Suitable vehicles for the emulsion layers and other layers of elements of this invention are described in Research Disclosure Item 17643, Section IX and the publications cited therein.

In addition to the couplers described herein the elements of this invention can include additional couplers as described in Research Disclosure Section VII, paragraphs D, E, F and G and the publications cited therein. These additional couplers can be incorporated as described in Research Disclosure Section VII, paragraph C and the publications cited therein.

The photographic elements of this invention can contain brighteners (Research Disclosure Section V), antifoggants and stabilizers (Research Disclosure Section VI), antistain agents and image dye stabilizers (Research Disclosure Section VII, paragraphs I and J), light absorbing and scattering materials (Research Disclosure Section VIII), hardeners (Research Disclosure Section XI), plasticizers and lubricants (Research Disclosure Section XII), antistatic agents (Research Disclosure Section XIII), matting agents (Research Disclosure Section XVI) and development modifiers (Research Disclosure Section XXI).

The photographic elements can be coated on a variety of supports as described in Research Disclosure Section XVII and the references described therein.

Photographic elements can be exposed to actinic radiation, typically in the visible region of the spectrum, to form a latent image as described in Research Disclosure Section XVIII and then processed to form a visible dye image as described in Research Disclosure Section XIX. Processing to form a visible dye image includes the step of contacting the element with a color developing agent to reduce developable silver halide and oxidize the color developing agent. Oxidized color developing agent in turn reacts with the coupler to yield a dye.

Preferred color developing agents are p-phenylene diamines. Especially preferred are 4-amino-3-methyl-N,N-diethylaniline hydrochloride, 4-amino-3-methyl-N-ethyl-N-β-(methanesulfonamido)ethylaniline sulfate hydrate, 4-amino-3-methyl-N-ethyl-N-β-hydroxyethylaniline sulfate, 4-amino-3-β-(methanesulfonamido)ethyl-N,N-diethylaniline hydrochloride and 4-amino-N-ethyl-N-(2-methoxyethyl)-m-toluidine di-p-toluene sulfonic acid.

With negative working silver halide this processing step leads to a negative image. To obtain a positive (or reversal) image, this step can be preceded by development with a non-chromogenic developing agent to develop exposed silver halide, but not form dye, and then uniform fogging of the element to render unexposed silver halide developable. Alternatively, a direct positive emulsion can be employed to obtain a positive image.

Development is followed by the conventional steps of bleaching, fixing, or bleach-fixing, to remove silver and silver halide, washing and drying.

The following examples further illustrate this invention. In these examples, comparative couplers having the following structures were employed:

### Comparative Image Couplers

The structures of couplers for use in the elements of the invention are shown in Tables I and II above.

### EXAMPLES 1-5

Photographic elements were prepared with the following layers, in the order indicated, on a cellulose acetate film support:

Layer 1: Red sensitized AgBrI emulsion (having an average grain diameter of 0.52»m, 6.4 mole % I) (1.61g Ag/m², 2.69g gel/m²), cyan image coupler (see Table III) and cyan DIR coupler (see Table III). Equimolar quantities of image couplers were used in the elements and the DIR couplers were used in amounts that would give essentially the same density and gamma in each of the elements after exposure and processing.

Layer 2: Overcoat layer of gelatin (1.08 g/m²) and Hardener bisvinylsulfonylmethane coated at 1.75% by weight of total gelatin.

The dried coatings were exposed (1/15 sec.) to daylight through a graduated density step wedge and processed at 37.8°C, as follows:

### color developer composition:

Sharpness was evaluated by calculating AMT acutance values for a 35mm system, as described in J. SMPTE, 82, 1009 (1973). Larger values of AMT indicate a sharper image is obtained. The results are reported in Table III.

The above data show a clearly discernible improvement in sharpness is obtained when a DIR coupler is used in combination with a 4-equivalent cyan dye-forming phenolic coupler having a para-cyanophenylureido group in the 2-position, and a sulfo containing ballast in the 5-position (II-2) vs a phenoxy ballast (C-1) in the 5-position. A similar result is obtained with the 2-equivalent couplers II-1 and II-5 vs C-2. It should be noted that two-equivalent image couplers give better sharpness than do four-equivalent image couplers.

### EXAMPLES 6-7

Color photographic elements were prepared with the following layers, in the order indicated, on a cellulose acetate film support.

Layer 1: A slow cyan dye-forming layer comprising a blend of a red-sensitized 0.42»m silver bromoiodide emulsion (6.1 mol% I) at 1.29g Ag/m² and a red-sensitized 0.21»m AgBrI emulsion (4.8 mole% I) at 0.43g Ag/m², gelatin (2.69g/m²), a masking coupler 1-hydroxy-4-(4-[2-(8-acetamido-1-hydroxy-3,6-disulfonaphthyl)azo]phenoxy)-2-(Δ-[2,4-di-tert.-amylphenoxy]butyl)naphthamide dipyridine salt (0.041g/m²), a cyan dye-forming coupler (see Table IV) and a DIR coupler (see Table IV).

Layer 2: A fast cyan dye-forming layer comprising a 0.76»m silver bromoiodide emulsion (6 mole% I) at 1.08g Ag/m², gelatin (1.61g/m²), a cyan dye-forming coupler (see Table IV) and a DIR coupler (see Table IV).

Layers 3 and 4: Gelatin at 2.85g/m².

Layer 5: A gelatin overcoat layer (2.8g/m²) hardened with bisvinylsulfonylmethane at 1.75% by weight of total gelatin. Equimolar quantities of the image coupler (C-1 or II-1) were used and the quantity of DIR coupler (I-2) was chosen to give essentially the same density and gamma in the exposed and processed element.

The dried elements were exposed and processed as in the preceding examples.

The above data show that a combination of a DIR coupler such as II-2 with a phenolic cyan dye-forming coupler having both a p-cyanophenylureido group in the 2-position, and a sulfo-containing ballast in the 5-position provides a sharpness improvement in comparison to a similar coupler combination in which the cyan dye-forming coupler does not have a sulfo-ballast in the 5-position.

### EXAMPLES 7-21

Multicolor photographic elements were prepared having the following schematic structure. In this structure the numbers in parenthesis show the coverage in g/m².

The amounts of couplers in each of the cyan dye forming layers were chosen to give essentially the same density and contrast in the exposed and processed elements. The dried coatings were exposed (1/500 sec), through a graduated density step wedge (Wratten 29 filter), and processed for 3-1/4 minutes in the C-41 process described in the British Journal of Photography Annual, 1977, pages 201-205. The AMT acutance values for 35 mm film system were calculated as described in the previous example.

The data show that within each set one obtains an improvement in sharpness as evidenced by the increase in AMT values with the combinations of this invention compared with combinations using the comparison image coupler C-1.

## Claims

1. A color photographic element comprising a support and a silver halide emulsion layer characterized in that there is associated therewith
a DIR compound having the structure I: wherein:
CAR is a carrier moiety;
TIME is a timing group; and
INH is a development inhibitor moiety;
together with a cyan dye-forming image coupler having the structure II: wherein:
m is 0 or 1;
n is 0, 1 or 2;
Y is halogen, or sulfonyl;
Q is -O- or -NH-;
R¹ is an unsubstituted or a substituted, straight or branched chain alkyl group having from 1 to 20 carbon atoms, an unsubstituted or a substituted cycloalkyl group having from 3 to 8 carbon atoms in the ring, an alkylcarbonyl or an alkoxycarbonyl group having from 1 to 20 carbon atoms in the alkyl or the alkoxy moiety;
R² is as defined for R¹ or is hydrogen;
R³ is an unsubstituted or a substituted alkyl group having from 1 to 24 carbon atoms, an unsubstituted or a substituted cycloalkyl group having from 3 to 8 carbon atoms in the ring, an unsubstituted or a substituted aryl group having from 6 to 24 carbon atoms, or an unsubstituted or a substituted heterocyclic group having from 3 to 8 atoms in the heterocyclic ring;
when R³ is a primary alkyl group, R¹ contains at least 2 carbon atoms;
Z is hydrogen or a coupling-off group; and the -CN substituent on the phenyl ureido group is para or meta to the ureido group.

2. A color photographic element of claim 1 wherein, in structure II, the cyano group is in the para position and n is 0.

3. A color photographic element of claim 2, wherein, in structure II, R¹ is alkyl of 1 to 20 carbon atoms and R² is hydrogen or alkyl of 1 to 4 carbon atoms.

4. A color photographic element of claim 2, wherein, in structure II, R¹ is alkyl of 1 to 14 carbon atoms, R² is hydrogen and R³ is alkyl of 2 to 24 carbon atoms.

5. A color photographic element of any one of claims 2 to 4, wherein, in structure I, CAR is a cyan or yellow dye-forming coupler moiety,
TIME has one of the structures: and where:
p is 1 to 4;
q is 0 or 1;
A is -O- or R⁵ is hydrogen, alkyl of 1-20 carbon atoms or aryl of 6 to 20 carbon atoms;
X is hydrogen and one or more substituents independently selected from hydroxy, cyano, fluoro, chloro, bromo, iodo, nitro, alkyl, alkoxy, aryl, aryloxy, alkoxycarbonyl, aryloxycarbonyl, carbonamido, and sulfonamido and
INH is a mercaptotetrazole inhibitor, or benzotriazole inhibitor or a oxadiazole inhibitor.

6. A photographic element of claim 5, wherein the DIR coupler has one of the structures: or wherein:
BALL is a ballast group;
R⁵ is hydrogen, alkyl of 1-20 carbon atoms or aryl of 6 to 20 carbon atoms;
INH is a mercaptotetrazole or a benzotriazole inhibitor;
X is hydrogen, cyano, nitro or sulfonamido;
p is 1-4 and
q is 0 or 1.

7. A photographic element of claim 1 wherein the cyan dye forming coupler has one of the structures:

8. A photographic element of claim 1, wherein the DIR compound is a coupler having one of the structures:

9. A color photographic element of claim 1, wherein the DIR compound is a cyan dye-forming DIR coupler and is contained in a red-sensitive silver halide emulsion layer together with the cyan dye-forming image coupler.

10. A color photographic element of claim 1, wherein the DIR compound is a yellow dye-forming DIR coupler and is contained in a red-sensitive silver halide emulsion layer together with the cyan dye-forming image coupler.

## Patentansprüche

1. Farbphotographisches Element mit einem Träger sowie einer Silberhalogenidemulsionsschicht, dadurch gekennzeichnet, daß dem Element zugeordnet ist eine DIR-Verbindung der Struktur I: worin bedeuten:
CAR einen Trägerrest;
TIME eine Zeitgebergruppe; und
INH einen Entwicklungsinhibitorrest;
gemeinsam mit einem einen blaugrünen Farbstoff bildenden Bildkuppler der Struktur II: worin bedeuten:
m gleich 0 oder 1;
n gleich 0, 1 oder 2;
Y Halogen oder Sulfonyl;
Q gleich -O- oder -NH-;
R¹ eine unsubstituierte oder eine substituierte, geradkettige oder verzweigtkettige Alkylgruppe mit 1 bis 20 Kohlenstoffatomen, eine unsubstituierte oder eine substituierte Cycloalkylgruppe mit 3 bis 8 Kohlenstoffatomen im Ring, eine Alkylcarbonyl- oder eine Alkoxycarbonylgruppe mit 1 bis 20 Kohlenstoffatomen in dem Alkyl- oder dem Alkoxyrest;
R² hat die für R¹ angegebene Bedeutung oder steht für Wasserstoff;
R³ eine unsubstituierte oder eine substituierte Alkylgruppe mit 1 bis 24 Kohlenstoffatomen, eine unsubstituierte oder eine substituierte Cycloalkylgruppe mit 3 bis 8 Kohlenstoffatomen im Ring, eine unsubstituierte oder eine substituierte Arylgruppe mit 6 bis 24 Kohlenstoffatomen oder eine unsubstituierte oder eine substituierte heterocyclische Gruppe mit 3 bis 8 Atomen im heterocyclischen Ring;
wobei gilt, daß wenn R³ eine primäre Alkylgruppe ist, R¹ mindestens 2 Kohlenstoffatome enthält;
Z Wasserstoff oder eine abkuppelnde Gruppe; und
der -CN-Substituent an der Phenylureidogruppe befindet sich in para- oder meta-Stellung zur Ureidogruppe.

2. Farbphotographisches Element nach Anspruch 1, bei dem in der Struktur II die Cyanogruppe sich in der para-Position befindet und n gleich 0 ist.

3. Farbphotographisches Element nach Anspruch 2, in dem in der Struktur II R¹ für eine Alkylgruppe mit 1 bis 20 Kohlenstoffatomen steht und R² für Wasserstoff oder eine Alkylgruppe mit 1 bis 4 Kohlenstoffatomen.

4. Farbphotographisches Element nach Anspruch 2, in dem in der Struktur II R¹ für eine Alkylgruppe mit 1 bis 14 Kohlenstoffatomen steht, R² für Wasserstoff und R³ für eine Alkylgruppe mit 2 bis 24 Kohlenstoffatomen.

5. Farbphotographisches Element nach einem der Ansprüche 2 bis 4, in dem in der Struktur I CAR für einen einen blaugrünen oder gelben Farbstoff bildenden Kupplerrest steht;
TIME eine der folgenden Strukturen aufweist: und worin bedeuten:
p gleich 1 bis 4;
q gleich 0 oder 1;
A gleich -O- oder R⁵ gleich Wasserstoff, eine Alkylgruppe mit 1 bis 20 Kohlenstoffatomen oder eine Arylgruppe mit 6 bis 20 Kohlenstoffatomen;
X gleich Wasserstoff und einen oder mehrere Substituenten, die unabhängig voneinander ausgewählt sind aus Hydroxy, Cyano, Fluoro, Chloro, Bromo, Iodo, Nitro, Alkyl, Alkoxy, Aryl, Aryloxy, Alkoxycarbonyl, Aryloxycarbonyl, Carbonamido und Sulfonamido, und worin
INH für einen Mercaptotetrazolinhibitor oder einen Benzotriazolinhibitor oder einen Oxadiazolinhibitor steht.

6. Photographisches Element nach Anspruch 5, in dem der DIR- Kuppler eine der folgenden Strukturen aufweist: oder worin bedeuten:
BALL eine Ballastgruppe;
R⁵ Wasserstoff, Alkyl mit 1 bis 20 Kohlenstoffatomen oder Aryl mit 6 bis 20 Kohlenstoffatomen;
INH einen Mercaptotetrazol- oder einen Benzotriazolinhibitor;
X gleich Wasserstoff, Cyano, Nitro oder Sulfonamido;
p gleich 1 bis 4; und
q gleich 0 oder 1.

7. Photographisches Element nach Anspruch 1, in dem der einen blaugrünen Farbstoff liefernde Kuppler eine der folgenden Strukturen aufweist:

8. Photographisches Element nach Anspruch 1, in dem die DIR-Verbindung ein Kuppler mit einer der folgenden Strukturen ist:

9. Farbphotographisches Element nach Anspruch 1, in dem die DIR-Verbindung ein einen blaugrünen Farbstoff liefernder DIR-Kuppler ist und in einer rot-empfindlichen Silberhalogenidemulsionsschicht gemeinsam mit dem den blaugrünen Farbstoff liefernden Bildkuppler enthalten ist.

10. Farbphotographisches Element nach Anspruch 1, in dem die DIR-Verbindung ein einen gelben Farbstoff liefernder DIR-Kuppler ist und in einer rot-empfindlichen Silberhalogenidemulsionsschicht zusammen mit dem den blaugrünen Farbstoff liefernden Bildkuppler enthalten ist.

## Revendications

1. Elément photographique en couleurs comprenant un support et une couche d'émulsion aux halogénures d'argent, caractérisé en ce qu'un coupleur DIR de structure I lui est associé : où :
CAR est un motif porteur ;
TIME est un groupe retardateur ; et
INH est un motif inhibiteur de développement ;
ainsi qu'un coupleur d'image formateur de colorant cyan de structure II : où :
m est 0 ou 1 ;
n est 0, 1 ou 2 ;
Y est un halogène, ou un groupe sulfonyle ;
Q est -O- ou -NH- ;
R¹ est un groupe alkyle à chaîne droite ou ramifiée, substitué ou non, de 1 à 20 atomes de carbone, un groupe cycloalkyle substitué ou non de 3 à 8 atomes de carbone sur le cycle, un groupe alkylcarbonyle ou alkoxycarbonyle de 1 à 20 atomes de carbone dans le motif alkyle ou alkoxy ;
R² est tel que défini pour R¹ ou est l'hydrogène ;
R³ est un groupe alkyle substitué ou non de 1 à 24 atomes de carbone, un groupe cycloalkyle substitué ou non de 3 à 8 atomes de carbone dans le cycle, un groupe aryle substitué ou non de 6 à 24 atomes de carbone, un groupe hétérocyclique substitué ou non de 3 à 8 atomes dans l'hétérocycle ;
lorsque R³ est un groupe alkyle primaire, R¹ contient au moins 2 atomes de carbone ;
Z est l'hydrogène ou un groupe se séparant au couplage ; et
le substituant -CN sur le groupe phényl uréido est en position para ou méta par rapport au groupe uréido.

2. Elément photographique en couleurs selon la revendication 1, dans lequel le groupe cyano de la structure II est en position para et n est égal à 0.

3. Elément photographique en couleurs selon la revendication 2, dans lequel R¹ de la structure II est un groupe alkyle de 1 à 20 atomes de carbone et R² est l'hydrogène ou un groupe alkyle de 1 à 4 atomes de carbone.

4. Elément photographique en couleurs selon la revendication 2, dans lequel R¹ de la structure II est un groupe alkyle de 1 à 14 atomes de carbone, R² est l'hydrogène et R³ est un groupe alkyle de 2 à 24 atomes de carbone.

5. Elément photographique en couleurs selon l'une quelconque des revendications 2 à 4, dans lequel CAR de la structure I est un motif de coupleur formateur de colorant cyan ou jaune,
TIME est représenté par l'une des structures : où :
p est de 1 à 4 ;
q est 0 ou 1 ;
A est -O- ou R⁵ est l'hydrogène, un groupe alkyle de 1 à 20 atomes de carbone ou un groupe aryle de 6 à 20 atomes de carbone ;
X est l'hydrogène ou un ou plusieurs substituants indépendamment choisis parmi les groupes hydroxy, cyano, fluoro, chloro, bromo, iodo, nitro, alkyle, alkoxy, aryle, aryloxy, alkoxycarbonyle, aryloxycarbonyle, carbonamido, et sulfonamido, et INH est un inhibiteur mercaptotétrazole, benzotriazole ou oxadiazole.

6. Elément photographique selon la revendication 5, dans lequel le coupleur DIR est représenté par l'une des structures : où :
BALL est un groupe ballast ;
R⁵ est l'hydrogène, un groupe alkyle de 1 à 20 atomes de carbone ou un groupe aryle de 6 à 20 atomes de carbone ;
INH est un inhibiteur mercaptotétrazole ou benzotriazole ;
X est l'hydrogène, un groupe cyano, nitro ou sulfonamido ;
p est de 1 à 4, et
q est 0 ou 1.

7. Elément photographique selon la revendication 1, dans lequel le coupleur formateur de colorant cyan est représenté par l'une des structures :

8. Elément photographique selon la revendication 1, dans lequel le composé DIR est un coupleur représenté par l'une des structures suivantes :

9. Elément photographique en couleurs selon la revendication 1, dans lequel le composé DIR est un coupleur DIR formateur de colorant cyan et est contenu dans une couche d'émulsion aux halogénures d'argent sensible au rouge avec le coupleur d'image formateur de colorant cyan.

10. Elément photographique en couleurs selon la revendication 1, dans lequel le composé DIR est un coupleur DIR formateur de colorant jaune et est contenu dans une couche d'émulsion aux halogénures d'argent sensible au rouge avec le coupleur d'image formateur de colorant cyan.
